

1

3,287,110

**NON-FERROUS ALLOY AND METHOD OF  
MANUFACTURE THEREOF**

Paul Joseph Scherbner, Boyertown, Pa., assignor to The Beryllium Corporation, Reading, Pa., a corporation of Delaware

No Drawing. Filed May 9, 1962, Ser. No. 193,588  
16 Claims. (Cl. 75—129)

This invention relates primarily to nickel-base alloys containing beryllium and to a process for producing the same. More specifically, the invention pertains to a new and improved melting procedure whereby nickel-base alloys containing beryllium along with titanium, aluminum, silicon, chromium, boron and zirconium may be produced without resorting to vacuum melting in order to produce ingots or billets for reduction by hot working or by casting. While the present invention will be described in relation to nickel base alloys, it will be understood that the teachings of the invention are equally applicable to cobalt and iron.

In the past, many problems have confronted the industry in the formation of nickel-base alloys containing beryllium because of the lack of a suitable, reliable, convenient and inexpensive method, that could be used industrially to produce high strength alloy material for engineering applications in relatively large melt sizes.

One of the main problems encountered by persons learned in the art of processing nickel-base alloys containing beryllium, was the occurrence of brittleness at elevated temperatures, of the order of 1200° F. or higher, during hot fabrication whenever the nickel alloys contained beryllium in excess of 1.7 percent and especially when the beryllium content was at 2 percent. Previously nickel-base alloys containing beryllium in excess of 1.7 percent could not be easily fabricated without cracking and without the prior necessity to prepare the alloy by vacuum melting, which is costly.

Because of the limitations in the prior art of melting nickel-base alloys containing beryllium, the commercial productivity and practical application of the high strength and corrosion-resistant properties of these nickel-base alloys with beryllium has been retarded by a capability of producing only relatively small ingots of less than 50 pound size, and that, only with the aid of a costly vacuum-melting procedure.

An object of the instant invention is to produce nickel-base alloys with beryllium for making ingots or billets for reduction by hot-working, as well as for castings without the necessity of vacuum melting.

A further object of the present invention is to set forth an improved process for producing nickel-base alloys containing beryllium in amounts of greater than 1.7% without the necessity of resorting to vacuum melting techniques.

A further object of the present invention is to set forth a process for producing nickel-base alloys containing beryllium wherein by adding certain elements in a specific and critical sequence during the melting operation, the hot workability of the alloy is improved without the necessity of resorting to vacuum melting techniques.

Another object of the instant invention is to introduce greater amounts of beryllium into wrought nickel alloys for strengthening purposes.

2

Yet another object of the instant invention is to produce a nickel-base alloy containing beryllium which can be easily fabricated without cracking and at the same time having high mechanical properties.

5 A still further object of the present invention is to produce a nickel-base alloy containing beryllium in amounts of greater than 1.7 percent capable of being hot-worked, cold-worked, and capable of developing through suitable heat treatment and precipitation hardening, high mechanical properties.

10 Yet another object of the instant invention is to set forth a process for making low-carbon nickel-beryllium alloys for cast or wrought applications wherein the alloy is capable of obtaining a high degree of hot and cold workability having significantly high tensile strength and hardness, after a precipitation hardening heat treatment.

15 Another object of the instant invention is to produce a nickel-base alloy which is capable of being cold-worked or formed to shape with ease and then strengthened later by aging.

20 Other objects and many attendant advantages of the invention will in part be obvious and in part appear hereinafter. For a further understanding of the nature and objects of the invention, reference should be had to the following detailed description.

25 There is provided by this invention an improved process for producing nickel-base alloys containing beryllium in amounts up to 3 percent, in melt quantities of the order of 30 500 pounds or more by using conventional industrial melting equipment without the need of resorting to the more costly procedure of melting under vacuum in order to be able to produce cast ingots or blanks for hot-processing, rolling, extrusion or forging and the like. This process is 35 also suitable for producing high strength, nickel-base alloys containing beryllium with other alloying elements, that are to be used in the form of castings in the heat-treated or unheat-treated conditions, or for making ingots for re-melt purposes. The material so produced is capable of being hot-worked, cold-worked and capable of developing through suitable heat-treatment and precipitation hardening, high mechanical properties.

40 On the basis of this invention, alloy compositions with 45 significantly high mechanical strength, in the fully heat-treated and aged condition, can be made in a wrought or cast condition and processed, consisting of the following elements within the composition ranges indicated in Table 1.

50

TABLE 1

| Element   | Minimum | Maximum |
|-----------|---------|---------|
| Beryllium | 0.6     | 3.0     |
| Titanium  | 0       | 4.5     |
| Silicon   | 0.1     | 1.0     |
| Aluminum  | 0.05    | 2.5     |
| Magnesium | 0.01    | 0.05    |
| Chromium  | 0       | 1.50    |
| 55 Boron  | 0       | 0.005   |
| Zirconium | 0       | 0.05    |
| Carbon    | 0       | 0.20    |
| Sulphur   | 0       | 0.002   |
| Nickel    | Balance |         |

With the exception of carbon and sulphur, which are considered to be undesirable commercial impurities in the alloys discussed, it is important to indicate the desirable presence in the alloy of small amounts of certain of the above elements, that when added in a specific and important sequence during the melting operation, contribute to improving the hot-workability of non-vacuum melted nickel-beryllium alloys.

Nickel-beryllium alloys containing substantial amounts of elements like titanium, aluminum, and chromium as shown in Table 1, can be melted in electric furnaces in air or preferably under a blanket of argon gas in order to minimize metal loss through oxidation. Illustratively, approximately 500 pounds of pure nickel metal, to which approximately 1 pound of carbon is added, is melted first and subjected to a carbon boil by adding nickel oxide powder to the molten nickel containing 0.20 percent carbon at a temperature of about 2800° F. The nickel oxide reacts with the carbon liberating carbon dioxide gases and carbon monoxide. The molten metal is stirred with a pure nickel rod until all reaction ceases, then a slight excess of additional nickel oxide is added. Any nickel oxide adhering to the pot or crucible is removed. It is, of course, understood that in the event the base melt is other than nickel, i.e., cobalt or iron, an oxide of cobalt or iron, as the case may be, would be added to the melt rather than nickel oxide.

Pure silicon metal (approximately 1.5 pounds) in the amount of 0.3 percent is next added to the melt in small pieces and stirred to react and chemically combine with the oxygen in the melt. The reaction between the oxygen and silicon is ended after a short time interval of a few minutes. The reaction product, which is a fluid slag, should be completely skimmed from the melt surface.

The temperature of the melt is maintained at 2600° F. to 2900° F. From this time on, an inert gas blanket is advantageously maintained over the surface of the melt until it is cast. The melt is stirred thoroughly once again to raise all the reaction product between the silicon and the oxygen to the surface of the melt for removal before other elements can be added. Next, 0.5 percent titanium may be added in the form of sponge to fulfill two functions: (1) to chemically combine with dissolved nitrogen gas that may have been absorbed during melting and to form small solid particles of titanium nitride dispersed through the alloy, and (2) the titanium in excess of that needed to combine with the dissolved nitrogen in order to form isolated particles of titanium nitride, serves to strengthen the alloy later by being available to form a precipitation hardening phase  $Ni_3Ti$ , or if aluminum is also present to form the compound  $Ni_3(Ti, Al)$ . If more than 0.4 to 0.5 percent titanium is desired in the alloy, then it is added later with the nickel-beryllium master alloy. After the addition of 0.5 percent titanium initially a characteristic surface

film but no slag, is formed on the melt surface. Then, 0.0025 percent boron in the form of 15 percent boron-nickel master and, 0.025 percent zirconium in the form of pure zirconium sponge are added to the melt to facilitate the hot-working characteristics of the alloy in the temperature range of 1700° to 1900° F. Magnesium, in the form of 10 percent magnesium-nickel master may also be added at the same time to combine with traces of any sulphur present in the alloy.

Up to this point, the alloying procedure has been to properly purify and condition the melt before the last additions of aluminum, chromium, titanium and finally beryllium in the form of 25 percent to 50 percent beryllium-nickel master alloy. After these additions are made, the metal temperature is raised to about 2700° F. and the alloy cast in a manner conventional with good foundry practice.

Many commercial nickel-base alloys without beryllium require substantial amounts of aluminum and titanium, ranging from 0-6 percent aluminum, and 0-4 percent titanium in order to maximize the age-hardening response. The addition of beryllium by lowering the solubility of both aluminum and titanium in the nickel matrix, permits smaller amounts of each of these elements to be required to produce maximum strengthening through aging, simultaneously allowing for easier cold deformation in the annealed condition because less solute atoms are in solution. The practical significance of this is realized since I have determined that nickel beryllium strip alloys with 3 percent titanium can be cold-worked with a 70 percent reduction in the area between anneals.

Specific examples of the versatility and capability of my process in producing high strength nickel-beryllium alloys with beryllium contents higher than heretofore claimed capable of being hot-worked or used as castings, without resorting to prior vacuum melting procedures are listed in the following cited examples. For simplification, the alloy compositions and mechanical properties obtained on representative samples of these particular alloys are identified by their respective heat numbers.

To indicate the versatility of the described process in producing wrought nickel-beryllium alloys with desirable mechanical properties, the alloys are arranged in the following groups:

- 45 Group I: Medium beryllium content (Be from 1 to 1.7%) and low titanium content (0 to 1% Ti). Heat No. 69.  
 Group II: High beryllium (Be from 1.70 to 2%), low titanium (Ti from 0 to 1%). Heat Nos. 50, 152.  
 Group III: High beryllium content (Be from 1.70 to 2%) and medium titanium content (Ti from 1 to 2%). Heat Nos. 160, 164.  
 Group IV: High beryllium content (Be ranging from 1.70 to 2%) and high titanium content (Ti ranging from 2 to 4.5%). Heat Nos. 36, 47, 48.  
 50 Group V: Medium beryllium content (Be—1.40%) and high titanium content (Ti—4.50%). Heat No. 109.

TABLE II.—COMPOSITIONS OF REPRESENTATIVE ALLOYS USED IN THIS INVENTION, PERCENT

| Heat No. | Be   | Ti   | Si   | Al   | Mg    | Cr    | B     | Zr    | C     | Ni   |
|----------|------|------|------|------|-------|-------|-------|-------|-------|------|
| 69       | 1.57 | 0.80 | 0.23 | 0.02 | 0.024 | 0.015 | 0.003 | 0.03  | 0.058 | Bal. |
| 50       | 1.91 | 0.66 | 0.31 | 0    | 0.024 | 0     | 0.002 | 0.015 | 0.010 | Bal. |
| 152      | 2.08 | 0    | 0.27 | 0.27 | 0.027 | 0.80  | 0.003 | 0.03  | 0.153 | Bal. |
| 160      | 1.71 | 2.00 | 0.06 | 0    | 0.025 | 0     | 0.003 | 0.03  | 0.071 | Bal. |
| 164      | 1.75 | 1.80 | 0.85 | 0    | 0.025 | 0     | 0.003 | 0.02  | 0.020 | Bal. |
| 47       | 1.67 | 3.06 | 0.30 | 0    | 0.029 | 0     | 0.003 | 0.05  | 0.019 | Bal. |
| 48       | 1.90 | 3.00 | 0.31 | 0.29 | 0.030 | 0.73  | 0.003 | 0.03  | 0.019 | Bal. |
| 36       | 1.74 | 3.14 | 0.35 | 0.38 | 0.047 | 0.78  | 0     | 0.055 | 0.018 | Bal. |
| 109      | 1.40 | 4.50 | 0.31 | 0    | 0.028 | 0     | 0.003 | 0.03  | 0.21  | Bal. |

TABLE III

|                                              | Heat No. | A*  | At  | H   | HT  | SH  | SHT |
|----------------------------------------------|----------|-----|-----|-----|-----|-----|-----|
| Ultimate Tensile Strength x 1,000 p.s.i.:    |          |     |     |     |     |     |     |
| Group I.....                                 | 69       | 86  | 171 | 146 | 245 |     |     |
| Group II.....                                | 50       | 96  | 211 | 153 | 282 | 177 | 284 |
|                                              | 152      | 108 | 255 | 170 | 286 |     |     |
| Group III.....                               | 160      | 113 | 233 | 155 | 265 |     |     |
|                                              | 164      | 110 | 229 | 174 | 291 |     |     |
| Group IV.....                                | 47       | 129 | 236 | 168 | 284 | 198 | 299 |
|                                              | 48       | 133 | 243 | 197 | 292 | 207 | 299 |
| Group V.....                                 | 36       |     | 246 |     | 275 | 210 | 291 |
|                                              | 109      | 135 | 231 | 197 | 273 |     |     |
| Yield Strength (0.2% offset) x 1,000 p.s.i.: |          |     |     |     |     |     |     |
| Group I.....                                 | 69       | 34  | 143 | 140 | 220 |     |     |
|                                              | 50       | 39  | 165 | 145 | 246 | 169 | 240 |
| Group II.....                                | 152      | 44  | 178 | 156 | 247 |     |     |
| Group III.....                               | 160      | 47  | 164 | 146 | 230 |     |     |
|                                              | 164      | 48  | 169 | 168 | 249 |     |     |
| Group IV.....                                | 47       | 62  | 168 | 159 | 236 | 188 | 260 |
|                                              | 48       | 62  | 167 | 184 | 246 | 197 | 262 |
| Group V.....                                 | 36       |     | 176 |     | 223 | 198 | 259 |
|                                              | 109      | 62  | 150 | 185 | 228 |     |     |

## \*Note:

A=Annealed,  $\frac{1}{2}$  hour at 1,900° F., and water quenched.AT=Annealed, water quenched, and aged,  $\frac{1}{2}$  hour at 1,000° F.

H=Annealed, water quenched, cold-rolled 37%.

HT=Annealed, water quenched, cold-rolled 37%, aged  $\frac{1}{2}$  hour at 1,000° F.

SH=Annealed, water quenched, cold-rolled 62%.

SHT=Annealed, water quenched, cold-rolled 62%, aged  $\frac{1}{2}$  hour at 1,000° F.

TABLE IV

|                                                   | Heat No. | A  | At  | H   | HT  | SH  | SHT |
|---------------------------------------------------|----------|----|-----|-----|-----|-----|-----|
| Proportional Limit (0.01% offset) x 1,000 p.s.i.: |          |    |     |     |     |     |     |
| Group I.....                                      | 69       | 20 | 88  | 84  | 165 |     |     |
|                                                   | 50       | 23 | 111 | 120 | 185 | 111 | 155 |
| Group II.....                                     | 152      | 27 | 129 | 118 | 145 |     |     |
|                                                   | 160      | 25 | 111 | 83  | 170 |     |     |
| Group III.....                                    | 164      | 33 | 109 | 117 | 123 |     |     |
|                                                   | 47       | 36 | 133 | 127 | 172 | 133 | 210 |
| Group IV.....                                     | 48       | 34 | 136 | 127 | 176 | 124 | 199 |
|                                                   | 36       |    | 115 |     | 175 | 114 | 198 |
| Group V.....                                      | 109      | 37 | 122 | 132 | 176 |     |     |
| Elongation, percent:                              |          |    |     |     |     |     |     |
| Group I.....                                      | 69       | 40 | 4   | 2   | 2   |     |     |
|                                                   | 50       | 43 | 6   | 4   | 4   | 2   | 11  |
| Group II.....                                     | 152      | 26 | 12  | 3   | 6   |     |     |
|                                                   | 160      | 41 | 14  | 4   | 2   |     |     |
| Group III.....                                    | 164      | 31 | 9   | 3   | 4   |     |     |
|                                                   | 47       | 33 | 15  | 5   | 8   | 1   | 4   |
| Group IV.....                                     | 48       | 28 | 15  | 4   | 10  | 1   | 7   |
|                                                   | 36       |    | 13  |     | 8   | 2   | 3   |
| Group V.....                                      | 109      | 32 | 20  | 2   | 11  |     |     |

TABLE V

|                | Heat No. | A   | At  | H   | HT  | SH  | SHT |
|----------------|----------|-----|-----|-----|-----|-----|-----|
| Rockwell:      |          |     |     |     |     |     |     |
| Group I.....   | 69       | 47B | 46C | 31C | 52C |     |     |
|                | 50       | 68B | 47C | 34C | 54C |     |     |
| Group II.....  | 152      | 68B | 64C | 38C | 55C |     |     |
|                | 160      | 75B | 50C | 34C | 56C |     |     |
| Group III..... | 164      | 71B | 51C | 38C | 56C |     |     |
|                | 47       | 89B | 49C | 38C | 54C | 43C | 55C |
| Group IV.....  | 48       | 90B | 48C | 40C | 54C | 43C | 56C |
|                | 36       |     | 60C |     | 54C | 45C | 56C |
| Group V.....   | 109      | 83B | 46C | 42C | 53C |     |     |

The alloys illustrated in the above examples show a lower yield strength and hardness in the annealed and cold-rolled condition than when aged. This is desirable in many applications and permits the alloys to be cold-worked or formed to shape with greater ease, then strengthened later by the aging treatment.

The addition of from 0.50 to 4.50 percent titanium and from 1 to 2 percent beryllium produces an alloy which not only has high hardness after aging, good elongation, high yield strength, but also good formability in the annealed condition. Also, the addition of 0.66% titanium to a nickel-base alloy containing 2% beryllium, can be produced by the disclosed process with resultant excellent fabricability as distinguished from the prior art.

Thus, by making use of the present invention, the alloys described can be hot- and cold-rolled with ease, without intercrystalline cracking, and with the desirable mechanical properties indicated in the above tables.

As this invention may be embodied in several forms without departing from the spirit or essential characteristics thereof, the present embodiment is therefore illustrative and not restrictive, and since the scope of the invention is defined by the appended claims, all changes that fall within the metes and bounds of the claims or that form their functional as well as conjointly cooperative equivalents are therefore intended to be embraced by those claims.

I claim:

1. A method of producing a nickel base alloy containing beryllium which comprises the steps of

- (1) melting said base metal in the presence of a quantity of carbon;
- (2) adding to the resulting melt a quantity of an oxide of said base metal to effect a first purification;
- (3) adding to said first purified melt a de-oxidizing agent sufficient to react and chemically combine with the oxygen of said melt;
- (4) removing from the melt the reaction product of the de-oxidizing agent and oxygen thereby effecting a second purification of the melt; and
- (5) adding to the melt the elements titanium, zirconium, aluminum, chromium and beryllium.

2. A method of producing a cobalt base alloy containing beryllium which comprises the steps of

- (1) melting said base metal in the presence of a quantity of carbon;
- (2) adding to the resulting melt a quantity of an oxide of said base metal to effect a first purification;
- (3) adding to said first purified melt a de-oxidizing agent sufficient to react and chemically combine with the oxygen of said melt;
- (4) removing from the melt the reaction product of the de-oxidizing agent and oxygen thereby effecting a second purification of the melt; and
- (5) adding to the melt the elements titanium, zirconium, aluminum, chromium and beryllium.

3. A method of producing an alloy containing beryllium and having as its base a metal selected from the group consisting of nickel, cobalt and iron, said method comprising the sequential steps of

- (1) melting said base metal with a quantity of carbon;
- (2) adding to the resulting melt a quantity of an oxide of said base metal sufficient to react therewith and cause the evolution of carbon dioxide and carbon monoxide thereby effecting a first purification;
- (3) adding to said first purified melt a quantity of silicon sufficient to react and chemically combine with the oxygen of said melt;
- (4) removing from the melt the reaction product of the silicon and oxygen thereby effecting a second purification of the melt;
- (5) adding up to 0.5% titanium to the melt to combine with any nitrogen gas present to form titanium nitride;
- (6) adding approximately 0.0025% boron;
- (7) adding approximately 0.025% of zirconium in the form of pure zirconium sponge;
- (8) finally adding to the melt the desired additional alloying elements including beryllium.

4. A method of producing an alloy containing beryllium as set forth in claim 3, wherein the base metal is nickel and wherein the oxide added in step (2) is nickel oxide.

5. A method of producing an alloy containing beryllium as set forth in claim 3, wherein the base metal is cobalt and wherein the oxide added in step (2) is an oxide of cobalt.

6. A method of producing an alloy containing beryllium as set forth in claim 3, wherein the base metal is iron and wherein the oxide added in step (2) is an oxide of iron.

7. A method of producing an alloy as defined in claim 3, wherein the ratio of addition of the carbon and silicon is approximately 1 pound carbon, one and a half pounds of silicon, and 500 pounds of base metal and wherein the temperature of the melt is maintained between about 2600° F. to 2900° F.

8. A nickel base alloy characterized by its susceptibility to fabrication without cracking and without the prior

necessity to prepare the same by vacuum melting, said alloy consisting of the following elements:

|                  | Percent   |
|------------------|-----------|
| Beryllium        | 0.6-3.0   |
| Titanium         | 0.0-4.5   |
| Silicon          | 0.0-1.0   |
| Aluminum         | 0.05-2.5  |
| Magnesium        | 0.01-0.05 |
| Chromium         | 0.0-1.50  |
| Boron            | 0.0-0.005 |
| Zirconium        | 0.0-0.05  |
| Nickel, balance. |           |

9. A nickel base alloy adapted to being produced without resorting to vacuum melting, consisting of:

|                  | Percent |
|------------------|---------|
| Beryllium        | 1.57    |
| Titanium         | 80      |
| Silicon          | 23      |
| Aluminum         | 0.2     |
| Magnesium        | .024    |
| Chromium         | .015    |
| Boron            | .003    |
| Zirconium        | .03     |
| Nickel, balance. |         |

10. A nickel base alloy adapted to being produced without resorting to vacuum melting, consisting of:

|                  | Percent |
|------------------|---------|
| Beryllium        | 1.91    |
| Titanium         | 66      |
| Silicon          | 31      |
| Magnesium        | .024    |
| Boron            | .002    |
| Zirconium        | .015    |
| Nickel, balance. |         |

11. A nickel base alloy adapted to being produced without resorting to vacuum melting, consisting of:

|                  | Percent |
|------------------|---------|
| Beryllium        | 2.08    |
| Silicon          | 27      |
| Aluminum         | 27      |
| Magnesium        | .027    |
| Chromium         | .80     |
| Boron            | .003    |
| Zirconium        | .03     |
| Nickel, balance. |         |

12. A nickel base alloy adapted to being produced without resorting to vacuum melting, consisting of:

|                  | Percent |
|------------------|---------|
| Beryllium        | 1.71    |
| Titanium         | 2.00    |
| Silicon          | .06     |
| Magnesium        | .025    |
| Boron            | .003    |
| Zirconium        | .03     |
| Nickel, balance. |         |

13. A nickel base alloy adapted to being produced without resorting to vacuum melting, consisting of:

|                  | Percent |
|------------------|---------|
| Beryllium        | 1.75    |
| Titanium         | 1.80    |
| Silicon          | .85     |
| Magnesium        | .025    |
| Boron            | .003    |
| Zirconium        | .02     |
| Nickel, balance. |         |

14. A nickel base alloy adapted to being produced without resorting to vacuum melting, consisting of:

|                  | Percent |    | Percent   |       |
|------------------|---------|----|-----------|-------|
| Beryllium        | 1.67    | 5  | Beryllium | 1.74  |
| Titanium         | 3.06    |    | Titanium  | 3.14  |
| Silicon          | .30     |    | Silicon   | 0.35  |
| Magnesium        | 0.29    |    | Aluminum  | 0.38  |
| Boron            | .003    | 10 | Magnesium | 0.047 |
| Zirconium        | .05     |    | Chromium  | 0.78  |
| Nickel, balance. |         |    | Zirconium | 0.055 |

15. A nickel base alloy adapted to being produced without resorting to vacuum melting, consisting of:

|                  | Percent |    | Percent          |       |
|------------------|---------|----|------------------|-------|
| Beryllium        | 1.90    | 15 | Beryllium        | 1.90  |
| Titanium         | 3.0     | 20 | Titanium         | 3.0   |
| Silicon          | 0.31    |    | Silicon          | 0.31  |
| Aluminum         | 0.29    |    | Aluminum         | 0.29  |
| Magnesium        | 0.030   |    | Magnesium        | 0.030 |
| Chromium         | 0.73    |    | Chromium         | 0.73  |
| Boron            | 0.003   | 25 | Boron            | 0.003 |
| Zirconium        | 0.03    |    | Zirconium        | 0.03  |
| Nickel, balance. |         |    | Nickel, balance. |       |

16. A nickel base alloy adapted to being produced without resorting to vacuum melting, consisting of:

|                  | Percent |   | Percent          |       |
|------------------|---------|---|------------------|-------|
| Beryllium        | 1.74    | 5 | Beryllium        | 1.74  |
| Titanium         | 3.14    |   | Titanium         | 3.14  |
| Silicon          | 0.35    |   | Silicon          | 0.35  |
| Aluminum         | 0.38    |   | Aluminum         | 0.38  |
| Magnesium        | 0.047   |   | Magnesium        | 0.047 |
| Chromium         | 0.78    |   | Chromium         | 0.78  |
| Zirconium        | 0.055   |   | Zirconium        | 0.055 |
| Nickel, balance. |         |   | Nickel, balance. |       |

#### References Cited by the Examiner

##### UNITED STATES PATENTS

|           |         |             |        |
|-----------|---------|-------------|--------|
| 1,941,368 | 12/1933 | Smith       | 75—170 |
| 2,062,130 | 11/1936 | Hessenbruch | 75—170 |
| 2,829,048 | 4/1958  | Cochardt    | 75—171 |
| 3,180,726 | 4/1965  | Nakamura    | 75—129 |

##### OTHER REFERENCES

"The Making, Shaping and Treating of Steel," Seventh edition, pages 352—353, published by United States Steel Corp.

25 DAVID L. RECK, *Primary Examiner.*

MARCUS U. LYONS, HYLAND BIZOT, *Examiners.*

R. O. DEAN, H. TARRING, *Assistant Examiners.*